

## UNITED STATES PATENT OFFICE

ADAM HOCHE, OF LYNN, MASSACHUSETTS, ASSIGNOR TO LITMO ADHESIVE & PRODUCTS COMPANY, OF LYNN, MASSACHUSETTS, A CORPORATION OF MASSACHUSETTS.

## PROCESS OF MAKING GLUE.

No Drawing.

Application filed October 11, 1922. Serial No. 593,882.

This invention has for its object to produce a glue which, on drying and setting, is waterproof. While the object of the invention is to provide a glue having this characteristic which is useful for a variety of purposes, nevertheless I have particularly in mind to produce a glue which is especially applicable for use in connection with gypsum in the manufacture of wall board or in 5 stucco work or in other kinds of work where-in gypsum is utilized. The raw material, which is employed in carrying out my process for the production of glue, is preferably chrome tanned leather, although of course it 10 will be understood that leather of other tannages may be utilized if desired.

The process, briefly stated, consists in 15 treating scraps or shavings of chrome tanned leather with baths of sulphuric acid of increasing dilution, so that the final product, while slightly acid, still contains a small proportion of chrome oxide which tans the gelatin, as the glue dries, to render the glue insoluble in water.

20 In carrying out this process, one may proceed as follows: The chrome tanned leather or leather scrap is immersed in a sufficient quantity of sulphuric acid of about 20° Bé. to cover it, and the mixture is stirred together and permitted to stand for a half an hour 25 more or less according to the size of the pieces of leather. The liquor is then drained off, carrying with it a portion of the extracted chrome oxide and is retained for the initial treatment of the next batch of leather. The 30 leather scrap is then immersed in a sulphuric acid solution of about 10° Bé. The leather is permitted to remain in this bath with stirring for half an hour more or less, whereupon 35 the liquor is drained off with such chrome oxide as may pass off therewith; and then the scrap is treated with a sulphuric acid solution of about 5° Bé. After thoroughly stirring for half an hour more or less, the liquor is 40 drawn off as thoroughly as can be effected. In this state, the leather scrap or particles of leather retain their shape. Then a small quantity of cold water is added so as to just 45 cover the scrap, and the scrap with the con-

tained water is then heated in a hot-water 50 bath until the leather is entirely dissolved. A glue is thus produced which is acid in reaction and in which sufficient chrome oxide is left, so that as the glue dries the gelatin is 55 tanned thereby, thus making the glue insoluble in water as previously stated. Whereas the leather scrap contains originally, say, 2% to 5% of chrome oxide, the final glue contains about 5/10% chrome oxide.

A glue, produced as thus described, may be 60 used as an adhesive for gluing wood, for pasting sheets of paper, boxboard, labels or the like, and may also be used as a size in the manufacture of certain papers or wall boards. In fact, it may be used for most of the 65 purposes for which an ordinary glue is employed where its acidity is not detrimental. It may be mixed with clay for the manufacture of fire bricks, or with wood pulp, sawdust, infusorial earth or other suitable filler in the 70 manufacture of molded articles. It is especially adapted for use with gypsum in the manufacture of gypsum board or in stucco work. In the manufacture of gypsum board, the gypsum is mixed with the glue instead 75 of with water, thereby forming a thicker paste which is more easily worked, and which is spread in a thick layer on a sheet of paper or paper board, and in some cases a surface 80 layer of paper or board is laid thereon. The glue, being acid, does not react with the gypsum, which itself is a sulphate. The result is that the acid glue prevents the gypsum from setting too rapidly and at the same 85 time forms a perfect adhesive for bonding the gypsum to the layer or layers of paper board, and renders the gypsum itself substantially waterproof.

What I claim is:

1. A process of making glue from chrome-tanned leather, which comprises extracting only a major portion of the chrome compound from the leather in successive baths of dilute sulphuric acid of successively decreasing acidities, and then heating the extracted 90 leather in water until it dissolves therein to form a waterproof glue containing a substantial amount of chrome oxide.

2. A process of making glue from chrome-tanned leather containing 2% to 5% chrome oxide, which comprises extracting the leather at room temperature in successive baths of 5 sulphuric acid of about 20° Baumé, about 10° Baumé and 5° Baumé, each extraction being performed for about half an hour, and

then heating the extracted leather in water until the leather dissolves in the water to form a waterproof glue containing a substantial amount of chrome oxide. 10

In testimony whereof I have affixed my signature.

ADAM HOCHE.